

## UNITED STATES PATENT OFFICE

2,576,847

PYRANTHRONE DYE COMPOSITIONS AND  
PROCESS FOR DYEINGJerry M. Mecco, Somerville, N. J., assignor to  
American Cyanamid Company, New York, N. Y.,  
a corporation of MaineNo Drawing. Application November 30, 1949,  
Serial No. 130,359.

18 Claims. (Cl. 8—34)

1

This invention relates to an improved process of dyeing with pyranthrone and its halogenated derivatives.

Pyranthrone (C. I. 1096) has the following formula:



and it, and its dibromo derivative (C. I. 1098) are well known vat dyes of golden-orange color. When these dyes are dyed by ordinary vat dyeing processes, which involve a strong alkali, such as sodium hydroxide and a reducing agent, such as sodium hydrosulfite, there is a loss in strength and brilliance, when the dyeing operation is carried out at high temperatures. On the other hand, high temperature dyeing presents such large practical economic advantages, that the properties of these two dyes, for dyeing at high temperatures, approaching that of boiling water, has hampered their economic exploitation.

High temperature dyeing usually improves dye penetration, and/or levelness, particularly with such fabrics as nylon. The fast-dyeing which is possible at high temperatures also makes various continuous and semi-continuous processes possible.

In referring to a "dye bath" it should be understood that we are considering the situation at the time the dye is affixed to the fabric. In many processes the dyestuff is present in a dye bath or vat in solution in the form of the reduced leuco compound, and the goods are introduced into this bath. In other processes, such as, for example, pigment dyeing processes, which lend themselves to continuous and semi-continuous processes of the package dyeing variety, the dyestuff may be originally incorporated loosely in the fiber in the form of a pigment and then reduced by the dye bath which contains only the reducing constituents and the caustic alkali which is necessary. In such a case, the dye bath at the fiber includes the dyestuff, but includes it actually in position in the fiber. Throughout this case, the term "dye

2

bath" will be used to cover both types of situation.

This invention is based on the discovery that when certain nitrogen compounds are incorporated into the vat dye bath, improved strength and brightness are obtainable in high temperature dyeing with pyranthrone, such as pyranthrone and dibromopyranthrone.

These nitrogen compounds, for the most part 10 organic in nature, are characterized by the fact that they contain a nitrogen atom united with at least one covalence bond to oxygen and with at least one covalence bond to an element other than oxygen or nitrogen. In the case of the organic 15 compounds, these are, for the most part, nitro and nitroso compounds, such as nitro-aliphatic, and nitro aromatic compounds, and the like. The few nitrogen compounds containing no carbon are, for the most part, hydroxyl amine and its derivatives, such as hydroxyl amine disulfonic acid. The various nitrogen compounds all exert some 20 beneficial effect. There is, however, a variation in the effectiveness of the individual compounds. Among the most powerful are nitropropane and 25 hydroxylamine, and as these compounds are readily obtainable at moderate cost, they present a definite economical advantage. Nitrobenzene is almost as effective, and its even lower cost also makes it a desirable material to use.

It is not known how the nitrogen compounds 30 operate in preventing loss of strength and brilliance in high temperature dyeing with pyranthrone; and, accordingly, the present invention is not intended to be limited to any theory of 35 action. In particular, the phenomena which underlie the present invention are all the more mysterious, because, as is described and claimed in my copending application Serial No. 130,355, filed November 30, 1949, nitrogen compounds exert a similar action with vat dyestuffs which are sensitive to over reduction or decomposition at high 40 temperatures. In the case of these dyes, which are easily decomposed or over reduced, it is possible that the nitrogen compounds may act as some kind of a reduction buffer. In the case of 45 pyranthrone and its halogenated derivatives, however, such an explanation is not tenable, because it is a known characteristic of these dyes that they do not show any appearance of decomposition or over reduction in baths up to the boiling 50 point of water. In spite of this well known stability of the dyestuffs, the nitrogen compounds exert their beneficial action to a marked degree. It is obvious that factors other than prevention of 55 over reduction or decomposition at high temper-

atures must be involved. What these other factors are, however, has still not been determined.

The advantages of the present invention are obtained both with pyranthrone and its halogenated derivatives. The degree of improvement, however, is considerably greater with dibromo-pyranthrone than with pyranthrone itself.

It is an advantage of the present invention that the amount of the nitrogen compounds to be used is not critical. There is, of course, a lower limit, and it has been found that when the amount of the nitrogen compounds is less than one-quarter by weight of the content of actual dyestuff in the bath, the improvements are not sufficiently marked to be of practical value. Above this minimum, results improve for a while, with increasing amounts of nitrogen compounds, but soon reach the point at which greater amounts of nitrogen compounds do not give any improvement. This point is approximately 16 parts by weight of the nitrogen compounds to 1 of dye. However, for practical operation, the improvement obtained with much smaller amounts (for example, from 1 to 3 parts of the nitrogen compounds per part of dye) so closely approaches the maximum improvement obtainable, that larger amounts of nitrogen compounds do not produce sufficient improvement to justify the additional cost. Even the upper limit of 16 parts of nitrogen compounds does not represent the maximum amount which can be used, without destroying the improvement in strength and brilliance, which is the purpose of the present invention. Even when 50 parts of nitrogen compounds to 1 part of dye are used, the improvements are still to be noted; but, of course, such enormous amounts of nitrogen compounds are only of theoretical interest.

Another advantage of the present invention is that the manipulative techniques of high temperature dyeing are not, in any way, changed by its use. Dyeing conditions remain the same, as do dyeing times; and the only change is that the shades obtained are stronger and brighter.

The optimum amount of nitrogen compounds to be used depends, to some extent, on the temperature of the dye bath and on the time during which dyeing takes place. In general, the faster the dyeing, the smaller the amount of nitrogen compounds which can be used to give results so closely approximating the optimum results, as to make larger amounts of nitrogen compounds practically unnecessary. When dyeing time is longer, as is customary, additional amounts of hydrosulfite are added to make up for hydrosulfite oxidized by the air, or by other factors.

It is an advantage of the present invention that it may be applied in several ways. For example, vat dye baths can be made up by adding all of the ingredients, that is, dye, alkali, reducing agent and nitrogen compounds, to produce a finished bath. Another method which has the practical advantage of making it unnecessary for the dyer to control closely the proportion of all ingredients going into the dye bath, is to blend with the dyestuff a suitable amount of nitrogen compounds to form a powder or a paste. This blend, which constitutes a new article of manufacture included within the scope of the present invention, may be sold. The dyer may then prepare his bath with the dyestuff blend, the alkali and the reducing agent in any convenient order.

The invention will be illustrated in greater de-

tail in conjunction with the following specific examples. Parts are by weight.

#### EXAMPLE 1

10 parts of cotton yarn was dyed in a bath containing about 0.09 part of the real dye having Color Index No. 1098, 3 parts of sodium hydroxide, 3 parts of sodium hydrosulfite, 1.5 parts of nitropropane in 400 parts of water. The bath was heated for 5 minutes at about 200° F. during which time the vat dye was reduced, after which the cotton yarn was entered and dyed for 60 minutes at about 200° F. The dyed yarn was then removed, and the excess dye liquor extracted from the yarn. The remaining dye on the yarn was then oxidized for five minutes in the air at room temperature, after which it was immersed in an oxidizing solution consisting of 0.1% glacial acetic acid solution and 0.1% sodium peroxide (100 volumes) for 10 minutes at 140° F. The dyed yarn was then rinsed in warm water to remove the excess acid, soaped at the boil for 10 minutes in 0.1% soap and 0.1% soda ash solution, rinsed and dried. The color was a bright orange and the yarn was dyed a full shade.

A second dyeing was made like the above except the 1.5 parts of nitro-propane were omitted from the dye bath. The material dyed in this bath was dull, weak and yellow.

#### EXAMPLE 2

The procedure of the preceding example was repeated except the dye having Color Index No. 1096 and 1.5 parts of sodium hydrosulfite were added after 5 minutes and another 1.5 parts were added after 20 minutes. The color value of the yarn dyed in this dye bath is a much stronger and brighter orange than that of the yarn dyed in the control sample in which no nitro-propane is present.

#### EXAMPLE 3

10 parts cotton yarn were dyed in a bath containing 0.9 parts of the real dye having Color Index No. 1096, 3 parts of sodium hydroxide, 3 parts of sodium hydrosulfite, 1.5 parts of para chloro ortho nitraniline in 400 parts of water. The bath was reduced for 5 minutes at 95° C. after which the cotton yarn was entered and dyed for 60 minutes at 95° C. The dyeing was bright orange and the yarn was dyed a full shade.

A second dyeing was made exactly as above except the 1.5 parts of para chloro ortho nitraniline were omitted from the dye bath. The cotton yarn dyed in this bath was a weaker shade of orange.

#### EXAMPLE 4

The procedure of the preceding example was repeated except the dye having Color Index No. 1098 and 1.5 parts of sodium hydrosulfite were added after 5 minutes and another 1.5 parts were added after 20 minutes. The color value of the yarn dyed in this dye bath is a much stronger and brighter orange than that of the yarn dyed in the control sample in which no para chloro ortho nitraniline is present.

#### EXAMPLE 5

The procedure of Example 1 was repeated except the 1.5 parts of nitro-propane were replaced with 1.5 parts of hydroxylamine hydrochloride. Again the dyeing was a bright orange with a nice red shade as compared to the dull yellower shade obtained in the control dyeing.

## 5

## EXAMPLE 6

The procedure of the preceding example was repeated except the 1.5 parts of hydroxylamine hydrochloride were replaced with 1.5 parts of nitrobenzene potassium sulfonate. The results were similar to those obtained in the preceding example.

## EXAMPLE 7

The procedure of the preceding example was repeated except the 1.5 parts of nitrobenzene potassium sulfate were replaced with 1.5 parts of nitrobenzene and after 15 minutes an additional 1.5 parts of sodium hydrosulfite were added. The shade of this dyeing was a nice strong orange showing that decomposition had not occurred as in the control sample.

## EXAMPLE 8

The procedure of the preceding example was repeated except the 1.5 parts of nitrobenzene were replaced with 1.5 parts of para-nitroacetanilide. The results were very similar to those obtained in the preceding example.

## EXAMPLE 9

The procedure of the preceding example was repeated except the para-nitroacetanilide was replaced with 1.5 parts of orthonitroso meta cresol. The yarn dyed in the bath containing the orthonitroso meta cresol was redder and brighter than the shade of the sample dyed in the control bath.

## EXAMPLE 10

The procedure of Example 1 was repeated except the compound  $\text{HON}(\text{SO}_3\text{K})_2 \cdot 2\text{H}_2\text{O}$  was used instead of the nitro-propane of Example 1. This compound was prepared as follows:

*Preparation of  $\text{HON}(\text{SO}_3\text{K})_2 \cdot 2\text{H}_2\text{O}$* 

42.5 parts potassium nitrite (0.5 mole) and 50 parts potassium acetate were dissolved in 100 parts of ice water. This was placed in a 3-neck flask fitted with a stirrer. 750 parts of finely chipped ice were added and the stirrer started.  $\text{SO}_2$  gas was passed into this mixture until an excess was added, as indicated by the effluent gas discoloring a dilute potassium permanganate solution. The temperature was kept around 0° C. during the reaction. The crystals of  $\text{HON}(\text{SO}_3\text{K})_2 \cdot 2\text{H}_2\text{O}$  were filtered with a Büchner funnel and the precipitate washed with four portions of ice water, each amounting to 25 parts, to remove sulfite and acetate. The precipitate was not dried, but stored damp in a refrigerator. Reference: Rollesson and Oldershaw, J. Am. Chem. Soc. 54, 977 (1932). The yarn dyed in the presence of the  $\text{HON}(\text{SO}_3\text{K})_2 \cdot 2\text{H}_2\text{O}$  was a brilliant orange of excellent strength as compared to the dull and yellower shade of the control dyeing.

## EXAMPLE 11

3 parts of the dye used in Example 1 and containing about 19% real dye was mixed with 3.0 parts of nitro-propane. The mixture was then added to 1170 parts of water at 160° F. To this was added 36 parts of 30° Bé. sodium hydroxide, after which the temperature was again adjusted to 160° F. and 9 parts of sodium hydrosulfite added and dissolved. The temperature was maintained at 160° F. for 15 minutes, after which time the color was reduced. This will be referred to as the standard leuco solution. 400 parts of this reduced dye solution were then transferred to a separate dye beaker.

## 6

20 parts of natural cotton yarn were pre-wet with approximately 1/2% solution of a pine oil soap, the excess removed by squeezing and the yarn then entered into the 400 parts of reduced vat dye and dyed at 160° F. for 45 minutes. The dyed yarn was then removed and the excess dye liquor extracted from the yarn. The remaining dye on the yarn was then oxidized for 5 minutes in the air at room temperature, after which it was immersed in an oxidizing solution consisting of 0.1% sodium peroxide and 0.1% glacial acetic acid solution for 10 minutes at 140° F. The dyed yarn was then rinsed in warm water to remove the excess glacial acetic, soaped at the boil for 10 minutes in 0.1% soap and 0.1% soda ash solution, rinsed and dried. A control dye bath was prepared exactly like the above except the nitro-propane was omitted. This was used to make a control dyeing using the same procedure as above. The yarn dyed in the bath containing the nitro-propane was stronger and brighter than the yarn dyed in the control dye bath.

## EXAMPLE 12

25 The procedure of the preceding example was repeated except the dyeing time was 1 hour and 45 minutes. The yarn dyed in the bath containing the nitro-propane showed an even greater increase in strength and brightness of shade as compared to the control dyeings than that obtained in the preceding example.

## EXAMPLE 13

35 The procedure of Example 1 was repeated except rayon was used in place of the cotton and the results were essentially the same as those obtained in Example 1.

## EXAMPLE 14

40 The procedure of the preceding example was repeated except linen was used in place of the rayon, and the results were substantially the same as those obtained when the rayon was used.

## EXAMPLE 15

45 The procedure of the preceding example was repeated except nylon was used in place of the linen. Quite unexpectedly the nylon was dyed a bright, strong shade of unusually level appearance and not the dull yellow shade obtained when no nitro-propane was present in the dye bath.

## EXAMPLE 16

55 The procedure of Example 1 was repeated except 0.025 part of the nitro-propane were used instead of the 1.5 parts of Example 1. The improvement in shade and brightness of this dyeing was definite but was not as pronounced as that obtained in Example 1.

## EXAMPLE 17

60 The procedure of Example 1 was repeated except the nitro-propane was replaced with N-(2-nitro-2-methyl-propyl) sulfanilic acid. The dyeing made from the bath containing the nitrogen compound was a bright, strong, reddish orange shade as compared to a dull, yellower shade for the control dyeing.

## EXAMPLE 18

65 A dyeing was made at a temperature of about 150° F. (approximately 50 pounds' pressure) on 2.5 parts of 80 x 80 bleached unmercerized cotton in the apparatus described in U. S. P. 75 2,405,167, using a dye bath containing 0.09 part

7

of real dye having Color Index No. 1098, 1 part of the nitrogen compound described in the preceding example, 5.0 parts of sodium hydroxide and 6 parts of sodium hydrosulfite, the dyeing being carried out in a dye bath having 300 parts of liquor for 2 minutes. The bath was then flushed with water to the sewer, the dyeing removed, oxidized and finished as in Example 1. A good, strong, bright red shade of orange was obtained. A control dyeing in which no N-(2-nitro-2-methyl-propyl) sulfanilic acid was present but otherwise made as above was a dull yellow shade.

## EXAMPLE 19

The procedure of the preceding example was repeated except a piece of nylon was used instead of a piece of cotton. The results were similar to those given in Example 18.

## EXAMPLE 20

500 parts of No. 20's, 2-ply, natural cotton yarn in package form were wet out with 7,000 parts of a  $\frac{1}{4}\%$  solution of the surface-active anionic material which had been preheated to 190° F. This was then dyed in a dye bath containing 9 parts of real dye having Color Index No. 1098, 15 parts of a surface-active anionic material and 22.5 parts of N-(2-nitro-2-methyl-propyl) sulfanilic acid in 1,000 parts of water, making a total dye bath of 8,000 parts.

The dye dispersion was first heated to 190° F. and then circulated through the wet-out package for 10 minutes, after which 200 parts of 30° Be. sodium hydroxide, which had been preheated to 190° F., were added to the dye bath and circulated for 5 minutes, after which 50 parts of solid sodium hydrosulfite were added and circulated for 25 minutes. The spent dye bath was then flushed from the machine. The dye was oxidized with 2% of 100-volume hydrogen peroxide for 10 minutes at 140° F., after which the package was soaped, rinsed and dried. A bright reddish orange dyeing having excellent levelness was obtained.

A control dyeing was made in the same manner except the nitrogen compound was omitted from the dye bath. The package dyed in the control bath was an uneven, dull yellowish shade.

## EXAMPLE 21

900 parts of the real dye, having Color Index No. 1098, were ground and dry blended with 250 parts of N-(2-nitro-2-methyl-propyl) sulfanilic acid. Ten parts of cotton were dyed in a bath containing 0.115 part of this blend, 3 parts of sodium hydroxide, and 3 parts of sodium hydrosulfite in 400 parts of water using the general method of Example 1. The resultant dyeing was stronger, redder and brighter than a control dyeing made from a bath containing the same amount of real dye, alkali and hydrosulfite but omitting the N-(2-nitro-2-methyl-propyl) sulfanilic acid.

## EXAMPLE 22

450 parts of the real dye of the preceding example were ground and dry blended with 7,500 parts of p-nitro-acetanilide. Ten parts of cotton yarn were dyed in a bath containing 1.6 parts of this blend, 3 parts of sodium hydroxide and 3 parts of sodium hydrosulfite in 400 parts of water using the general method of the preceding example. The dyeing obtained from this dye bath was stronger and brighter than that obtained from a control dye bath in which no p-nitroacetanilide was present.

8

## EXAMPLE 23

960 parts of the dye having Color Index No. 1096 and 2,400 parts of HON(SO<sub>3</sub>K)<sub>2</sub>·2H<sub>2</sub>O were ground and dry blended to give a homogeneous mixture. Ten parts of rayon yarn were dyed in a bath containing 0.35 part of this blend, 3 parts of sodium hydroxide, and 3 parts of sodium hydrosulfite in 400 parts of water by the general method used in Example 1. The yarn dyed in the bath containing the HON(SO<sub>3</sub>K)<sub>2</sub>·2H<sub>2</sub>O was redder and brighter than the control dyeing.

## EXAMPLE 24

460 parts of a 20% wet press cake containing 92 parts of the real dye used in Example 21 and 25 parts of hydroxylamine hydrochloride were stirred together and made up to 1,000 parts with water. One part of this aqueous paste was substituted for the 0.115 part of dry blended material of Example 21, the dyeing being made as in Example 21. The dyeing made from the bath containing the hydroxylamine hydrochloride was stronger and brighter than that made from a control dye bath in which no hydroxylamine hydrochloride was present.

## EXAMPLE 25

462.5 parts of the 20% wet press cake containing about 92.5 parts of the dye having Color Index No. 1098 and 400 parts of nitro-benzene potassium sulfonate were stirred together and then made up to 1,000 parts with water. One part of this paste was substituted for the one part of the paste of the preceding example, the dyeings were made as in the preceding example, and the results were satisfactory.

## EXAMPLE 26

The procedure of the preceding example was repeated except part of the water needed to bring the paste to 1,000 parts was replaced with glycerine to give a glycerine content of 5%–10% on the final weight. Dyeings made with pastes containing glycerine were quite satisfactory.

## EXAMPLE 27

The procedure of the preceding example was repeated except the glycerine was replaced by ethylene glycol. Cotton yarn dyed with this paste is commercially satisfactory.

## EXAMPLE 28

The procedure of the preceding example was repeated except the wet press cake was dispersed with 10 parts of the sodium salt of di-sulfo-di-naphthyl methane, the humectant then added and the paste made up to 1,000 parts. Cotton yarn dyed in a bath containing one part of this paste but otherwise dyed as in Example 25 gave satisfactory results.

I claim:

1. A method of vat dyeing fibrous material to which alkali metal salts of the leuco vat pyranthrone dye are substantive with a pyranthrone dye, which comprises dyeing the material at high temperature approaching the boiling point of water in a bath containing the dyestuff, strong alkali, reducing agent, and an amount of a nitrogen compound, in which a nitrogen is attached by at least one covalence bond to oxygen and by at least one covalence bond to an element other than oxygen or nitrogen, equal to at least one-quarter the weight of the real dyestuff.

2. A method according to claim 1, in which the

nitrogen compound is N-(2-nitro-2-methyl-propyl) sulfanilic acid.

3. A method according to claim 2 in which the dyestuff is pyranthrone.

4. A method according to claim 2 in which the dyestuff is dibromopyranthrone.

5. A method according to claim 1 in which the dyestuff is pyranthrone.

6. A method according to claim 1 in which the dyestuff is dibromopyranthrone.

7. As a new article of manufacture a blend of a pyranthrone vat dyestuff with an amount of a nitrogen compound, in which a nitrogen is attached by at least one covalence bond to oxygen and by at least one covalence bond to an element other than oxygen or nitrogen, equal to at least one-quarter the weight of the real dyestuff.

8. An article of manufacture according to claim 7 in which the nitrogen compound is N-(2-nitro-2-methyl-propyl) sulfanilic acid.

9. An article of manufacture according to claim 8 in which the dyestuff is pyranthrone.

10. An article of manufacture according to claim 8 in which the dyestuff is dibromopyranthrone.

11. An article of manufacture according to claim 7 in which the dyestuff is pyranthrone.

12. An article of manufacture according to

claim 7 in which the dyestuff is dibromopyranthrone.

13. A method according to claim 1 in which the nitrogen compound is a nitroalkane.

14. A method according to claim 13 in which the nitroalkane is a nitropropane.

15. A method according to claim 1 in which the nitrogen compound is a hydroxylamine compound.

16. An article according to claim 7 in which the nitrogen compound is a nitroalkane.

17. An article according to claim 16 in which the nitroalkane is a nitropropane.

18. An article according to claim 7 in which the nitrogen compound is a hydroxylamine compound.

JERRY M. MECCO.

#### REFERENCES CITED

20 The following references are of record in the file of this patent:

#### UNITED STATES PATENTS

| Number    | Name       | Date          |
|-----------|------------|---------------|
| 2,029,999 | Grieshaber | Feb. 4, 1936  |
| 2,146,646 | Nusslein   | Feb. 7, 1939  |
| 2,383,393 | Kienle     | Aug. 21, 1945 |